

# UNITED STATES PATENT OFFICE.

ERNST HAMMESFAHR, OF SOLINGEN, NEAR FOCHE, GERMANY.

## METHOD OF MANUFACTURING CUTLERY.

No. 815,699.

Specification of Letters Patent.

Patented March 20, 1906.

Application filed November 4, 1901. Serial No. 84,491.

*To all whom it may concern:*

Be it known that I, ERNST HAMMESFAHR, a subject of the King of Prussia, German Emperor, residing at Solingen, near Foche, in the Kingdom of Prussia, German Empire, have invented a new and Improved Method of Manufacturing Cutlery, of which the following is a specification.

The object of the present invention is to minimize the time and labor required to turn out the finished article, at the same time securing greater uniformity of qualities and increased density throughout the article.

The articles to be formed are first roughly blanked out by ordinary forging. Then the prepared blank is again forged out, giving roughly the outlines of the article, and the necessary drawing or squeezing out of metal is practically completed. In the next forging the finished article is produced almost in its proper dimensions, but with a wide fin of superfluous metal. These forgings are done with the blanks at usual forging heat. The next operation consists in removing the hammer-scale or forge-scale. This is effected by subjecting the pieces to the abrading action of sharp sand or similar material in a revolving drum or by the known pickling process in the acid-bath. Next the fin along the cutting edge or edges of the article is cut off. It is not disturbed as yet along the remaining parts of the tool, such as the back of the blade or the tang. The reason is that it is intended to subject the piece to one cold-forging between the hot-forgings and then to another forging action, which is to be more of the nature of mere polishing than of forging or changing of shape in any way. During the cold-forging the blade proper will draw to some extent, and by cutting away the fin along the cutting edge only the flow of metal will be in that direction, which is as it should be. The cleansed pieces are now placed cold between highly-polished swages suitably shaped to bring out sharply all the contour of the finished article and there subjected to a cold-forging, the object of which is mainly to remove any irregularities remaining over from the hot-forging or which

may have been brought out by removing the hammer-scale, as would be the case if particles of scale had lodged in minute pockets, preventing uniformity of forging action. Now the entire fin is cut away. The piece is practically complete as to shape. The bur produced in cutting off the fin is next removed by again passing the piece through the abrading action of sand or emery in the revolving drum or equivalent means. The surfaces are next smoothed off and given a partial polish by again cold-forging them between highly-polished swages. This last action leaves the tool ready for tempering and the finishing-polish without any preceding grinding. It is to be noted that the successive forgings improve the quality of material, as well as the appearance of the surface.

Having now described my invention, what I claim, and desire to secure by Letters Patent, is—

1. The method of finishing cutlery without grinding, which consists in producing a keen edge by cold-swaging and then hardening and polishing.

2. The method of finishing cutlery without grinding, which consists in reducing the work-pieces by successive steps to the general form of the desired product, producing a keen edge by cold-swaging in highly-finished steel swages, and then hardening and polishing.

3. The method of working rough cutlery-blades, consisting in removing the scale from the rough blades; removing the excess of material at the cutting edge of the same; swaging them in a cold state in steel swages, removing the fin produced by said swaging; removing the bur resulting from removing said fin; swaging the thus-treated work-pieces in highly-polished steel swages; and hardening and polishing them, substantially as, and for the purpose described.

In witness whereof I have hereunto set my hand in presence of two witnesses.

ERNST HAMMESFAHR.

Witnesses:

ERNST KATZ,  
ANTON APEMACHER.